

# UNITED STATES PATENT OFFICE.

GALEN HOWELL CLEVENGER, OF PALO ALTO, CALIFORNIA, ASSIGNOR TO MERRILL METALLURGICAL COMPANY, A CORPORATION OF CALIFORNIA.

## PRECIPITANT FOR RECOVERING METALS FROM SOLUTIONS.

1,123,685.

Specification of Letters Patent.

Patented Jan. 5, 1915.

No Drawing.

Application filed June 11, 1912. Serial No. 702,973.

*To all whom it may concern:*

Be it known that I, GALEN HOWELL CLEVENGER, a citizen of the United States of America, and resident of Palo Alto, Santa Clara county, State of California, have invented new and useful Improvements in Precipitants for Recovering Metals from Solutions, of which the following is a specification.

10 My invention relates to an improvement in precipitants for recovering metals from solutions, and particularly to that class of precipitant which is employed for the purpose of precipitating precious metals from 15 cyanid solutions.

In practice, various forms of precipitants are used, but the most satisfactory and economical precipitants which have hitherto been employed in this art, are precipitants 20 composed of malleable metallic zinc in the form of either threads or spheres, the spheres composing what is known in practice as "zinc fume" or "zinc dust". On account of its malleability, metallic zinc 25 has hitherto resisted any form of mechanical comminution down to a powder which will expose sufficient surface to enable it to be used in a process of precipitation which involves agitation, conduction of the mixture, and the subsequent filtration thereof.

Now, I have discovered that where a precipitant is employed composed of a suitable alloy of zinc, which may be easily comminuted to an angular powder, and which is 35 introduced into the solution to be treated in such form, an economical, easily regulated, and metallurgically efficient precipitation results, which is free from the defects which have hitherto existed in precipitation 40 by metallic zinc. For this purpose I use preferably sodium as I find that it is the cheapest substance practicable and less likely to give trouble through the formation of insoluble compounds than other metals, 45 and at the same time gives the desired degree of brittleness. The alloy produced will have very much greater efficiency from a chemical point of view, as the presence of

the sodium, and possibly the lead in the alloy, bring about a quicker action and 50 necessitate the use of a smaller amount of precipitant, even though the mechanical subdivision remains approximately the same.

In practice, such a brittle alloy is composed of zinc, mixed preferably with not over three per cent. of sodium, or any other alkali or alkaline earth metal which will impart brittleness to the resultant alloy, or any one or more of these metals in suitable 60 proportions, dependent upon the character of the solution to be precipitated and the point of saturation of any particular metal in the alloy employed, and is prepared in any convenient form of reducing receptacle 65 in which they can be brought together. In practice, a vessel is used in which the alloy can be compounded with a minimum of oxidation. After the alloy is formed, and allowed to cool, it may be readily and quickly 70 reduced to an angular powder in any convenient form of comminuting apparatus.

The powder thus formed may be used as a precipitant in the place of the various forms of metallic zinc precipitants which 75 have hitherto been used in any of the well-known processes of cyanidation, according to the practice of these processes.

I claim as my invention:

1. A precipitant for recovering metals 80 from cyanid solutions, consisting of a binary brittle alloy of zinc with alkali or alkaline earth metal.

2. A precipitant for recovering metals 85 from cyanid solutions, consisting of a powder made from a brittle alloy, consisting of zinc and alkali or alkaline earth metal, susceptible of reduction to any degree of fineness.

3. A precipitant for the recovery of 90 metals from cyanid solutions, consisting of a brittle alloy of zinc and not more than three per cent. (3%) of alkali or alkaline earth metal.

4. A precipitant for the recovery of 95 metals from cyanid solutions, consisting of

a powder made from a brittle alloy, composed of zinc, and not more than three per cent. (3%) of sodium, for imparting brittleness to the said alloy, substantially as set forth.

In testimony, that I claim the foregoing as my invention, I have signed my name in

presence of two witnesses, this 18th day of April, 1912.

G. HOWELL CLEVENGER.

Witnesses:

C. C. BROADWATER,  
HERBERT S. SHUEY.